# EUROPEAN PATENT SPECIFICATION

(11) **EP 1 088 130 B1**
(45) Date of publication and mention of the grant of the patent: **31.03.2004**
(21) Application number: 98922379.7
(22) Date of filing: 15.05.1998
(51) Int. Cl.: D21C 9/10, D21C 9/16, D21C 9/147

(54) **PEROXIDE, OXYGEN, AND PEROXIDE/OXYGEN BRIGHTENING OF CHEMICAL AND MIXED WASTE PULPS**
PEROXIDE, SAUERSTOFF, UND PEROXIDE/SAUERSTOFF BLEICHEN VON ZELLSTOFFEN UND ALTPAPIERFASERSTOFFEN
ECLAIRCISSEMENT DE PATES CHIMIQUES ET DE PATES DE VIEUX PAPIERS MELANGES, AU MOYEN DE PEROXYDE, D'OXYGENE OU DE PEROXYDE/OXYGENE

(43) Date of publication of application: 04.04.2001
(73) Proprietor: National Silicates Partnership, Etobicoke, Ontario M8Z 5C7 (CA); The Research Foundation of State University of New York, Albany, NY 12246 (US)
(72) Inventor: EVANS, Timothy, D., Oakville, Ontario L6J 2T5 (CA); FRANCIS, Raymond, C., Dewitt, NY 13214 (US)
(74) Representative: Schwabe - Sandmair - Marx
(86) International application number: PCT/US1998/010070
(87) International publication number: WO 1999/060201

(56) References cited:
- EP-A- 0 148 712
- WO-A-94/10374
- US-A- 4 915 785

## Description

The present invention pertains to the brightening of chemical pulps and deinked, mixed office waste pulps, and particularly to the brightening of such pulps in a peroxide or peroxide/oxygen stage of brightening.

The process of making paper from wood involves the following general stages: (1) bark removal; (2) wood chipping; (3) pulping; (4) brightening; and (5) forming a sheet of paper on a machine. During pulping, wood is reduced to its fibrous state, with a portion of the lignin content in the wood being removed. Pulps can be divided into two main categories - chemical and mechanical pulps - depending on how they are made from wood. Chemical pulping involves the use of chemical reagents to effect a separation of the cellulose fibers from the other wood components, such as lignin and other extraneous compounds. In the process, most of the hemicelluloses are also dissolved. Thus, the yield for chemical pulping is typically 40-50 % on wood.

Mechanical pulping involves the reduction of wood to the fibrous state by mechanical means, such as by grinding logs into pulp by large revolving grindstones. These pulps are called "mechanical" because a significant amount of mechanical energy (grinding or refining) is required to break down the wood chips. Except for a few water soluble components, all of the constituents of the wood are present in the ground wood pulp. Thus, mechanical pulps are characterized by their high yield and high lignin content. For example, although chemical pulps contain only about 5% lignin (weight basis on pulp) after pulping, mechanical pulps typically contain greater than 20 % lignin for hardwoods and 25 % for softwoods after pulping.

In general, the brightening of chemical and mechanical pulps occur by different mechanisms. This difference in approach is due, in part, to the difference in lignin content between the chemical and mechanical pulps and to the different nature of the lignin in chemical pulps than that in mechanical pulps. The remaining lignin in chemical pulps is typically more difficult to degrade than the majority of the lignin remaining in mechanical pulps. For example, chemical pulps, such as kraft pulps, are more difficult to brighten by H₂O₂. Thus, instead of the 60°C bleaching temperature used for mechanical pulps, values in the range of 110°C are used for kraft pulps (which use sodium hydroxide and sodium sulfide as the primary chemical reagents). As another example of the differences in brightening the two different types of pulp, chlorine dioxide (ClO₂), a stable free radical, is involved in the brightening of more than 90 % of bleached kraft pulp produced in the U.S.A. per year. On the other hand, it has been reported that chlorine dioxide actually darkens mechanical pulps. In sum, results obtained with mechanical pulps cannot be considered as being predictive for chemical pulps.

Various additives have been proposed to improve the brightening process of mechanical pulps or mixed chemical/mechanical pulps having a high lignin content (i.e., above 20 % by weight on pulp). Sodium silicate is widely used for hydrogen peroxide brightening of such pulps. It acts as a peroxide stabilizer and as a buffer during the bleaching reaction. Sodium silicate, in combination with a small dose of MgSO₄, has long been known to improve the brightness of mechanical pulps. The two chemicals are known to form an intermediate that adsorbs or complexes transition metal species which would otherwise undesirably catalyze the decomposition of H₂O₂. The two chemical combination is widely used in installations that bleach mechanical pulps. When magnesium sulfate has been used for such pulps, however, no increase in brightness has been observed when the MgSO₄·7H₂O dose is increased above 0.05% on mechanical pulp (2.0 mmoles/kg). Accordingly, previous researchers had no need to add more magnesium to their pulps.

Turning to the brightening of chemical pulps, some results have suggested that silicate has a negative effect on H₂O₂ bleaching of kraft pulps. In some cases, the inclusion of silicate lowered the brightness by 4.6 percentage points (measured as % GE brightness in accordance with TAPPI Standard T452 om-92) and by 2-7 percentage points.

In peroxide brightening of mechanical pulps, the key is nucleophilic degradation of carbonyl compounds in the native lignin without the oxidation of phenols to o- and p- quinones, as shown below in reactions [A] and [B], respectively. Reaction [A] is the desirable degradation of carbonyl compounds by the perhydroxyl anion, OOH⁻. This reaction breaks down the carbonyl compounds, which absorb light in the visible range, to a more soluble form to be washed away by water. On the other hand, reaction [B] represents the undesirable formation of o- and p- quinones, which are less soluble in water and also absorb light in the visible range.

The perhydroxyl anion is generated by the dissociation of H₂O₂ as shown by equation [1] below. Mild conditions have to be used to prevent the oxidation of phenolics. ${\text{H}}_{\text{2}} {\text{O}}_{\text{2}} {\text{+ H}}_{\text{2}} {\text{O ↔ H}}_{\text{3}} {\text{O}}^{\text{+}} {\text{+ OOH}}^{\text{-}} \text{pKa = 11.6}$Mechanical pulps contain high concentrations of lignin and extractives whose negatively charged sites may complex transition metals. Also, some transition metal catalysis can be tolerated because lignin is a very good radical scavenger. It will scavenge the superoxide anion (· O₂⁻) and prevent wasteful decomposition to O₂ (equation [2]). ${\text{·O}}_{\text{2}} {\text{}}^{\text{-}} {\text{+ M}}^{\text{(n+l)+}} {\text{→ O}}_{\text{2}} \text{+} {\text{M}}^{\text{n+}}$Actually, · O₂⁻ is nucleophilic and its reaction with lignin is reported to result in increased brightness. In sum, transition metal deactivation by magnesium silicates is important but not critical to the brightening of mechanical pulps.

Unlike softwood mechanical pulps which typically contain about 25% lignin (by weight on pulp), chemical pulps enter the final brightening stage with typically less than 2 % lignin, which is typically colored and very difficult to oxidize. The approach with H₂O₂ is nucleophilic degradation by OOH⁻.
However, equation [2] becomes favorable because there is not a large amount of reactive lignin to scavenge · O₂⁻. Equation [2], in conjunction with equations [3] and [4], results in wasteful decomposition of H₂O₂. ${\text{M}}^{\text{n+}} {\text{+ H}}_{\text{2}} {\text{O}}_{\text{2}} {\text{→ M}}^{\text{(n+l)+}} {\text{+ ·OH+}}^{\text{-}} \text{OH}$${\text{·OH+}}^{\text{-}} {\text{OOH → ·O}}_{\text{2}} {\text{}}^{\text{-}} {\text{+ H}}_{\text{2}} \text{O}$Equation [3] is favorable for Cu(I) and Fe(II) but not for Mn(II). A more probable mechanism for Mn(II) is outlined below. The subscripted s indicates soluble Mn(IV) and Mn(III). ${\text{Mn}}^{\text{2+}} {\text{}}_{\text{(s)}} {\text{+ H}}_{\text{2}} {\text{O}}_{\text{2}} {\text{→ Mn}}^{\text{4+}} {\text{}}_{\text{(s)}} {\text{+ 2OH}}^{\text{-}}$${\text{Mn}}^{\text{4+}} {\text{}}_{\text{(s)}} {\text{+}}^{\text{-}} {\text{OOH → Mn}}^{\text{3+}} {\text{}}_{\text{(s)}} {\text{+ H}}^{\text{+}} {\text{+ ·O}}_{\text{2}} {\text{}}^{\text{-}}$${\text{Mn}}^{\text{3+}} {\text{}}_{\text{(s)}} {\text{+}}^{\text{-}} {\text{OOH → Mn}}^{\text{2+}} {\text{}}_{\text{(s)}} {\text{+ H}}^{\text{+}} {\text{+ ·O}}_{\text{2}} {\text{}}^{\text{-}}$Lignin degradation by OOH⁻ requires a high temperature because of the unreactive nature of the lignin in chemical pulps. At 110°C, transition metal deactivation is extremely important.

With respect to O₂ delignification, a simple and well-accepted scheme for free radical generation is provided below. RH is a reactive structure in the solution phase. ${\text{RH + O}}_{\text{2}} \text{→ R ·} \text{+} \text{· OOH}$${\text{· OOH + H · → HOOH (H}}_{\text{2}} {\text{O}}_{\text{2}} \text{)}$

(Abstraction of H atom from lignin) ${\text{R· +O}}_{\text{2}} \text{→ ROO ·}$$\text{ROO · + H · → ROOH}$H₂O₂ and ROOH will be affected by transition metals in the same manner as in a peroxide/oxygen stage. Thus, the oxygen stage is similar to the peroxide/oxygen stage in that they both involve heterolytic (i.e., ionic) reactions and homolytic (i.e., free radical) reactions. In addition, they are both similar in that both rely on hydrogen peroxide, either as added in the peroxide/oxygen stage or as generated in reaction [6] above in the oxygen stage, to perform a brightening function. It is assumed that organic peroxides (ROOH in equation [8]) generated during oxygen delignification dissociate to form ROO⁻ nucleophiles that brighten lignin.
Accordingly, in both stages (as well as in a peroxide stage), one must be concerned about transition metals undesirably catalyzing free radical reactions.

EP-A-0 148 712 discloses a process for bleaching of chemical pulps by using hydrogen peroxide at an elevated pH of 11 to 11.5, and a temperature of 70°C to 100°C in presence of an amount of alkali metal silicate such that the concentration of silicon oxide in the pulp is at least 0.3 wt-%, and that the amount of magnesium or calcium salts is in the range between 0.05 wt-% and 1 wt-%. The process is characterized in that the pulp also comprises a chelating agent for the alkaline earth metals, which chelating agent is used in an amount of 10 wt-% or more.

WO 94/10374 discloses a process for peroxide bleaching of sulfite cellulose which has been prebleached in an acid oxidative step and thereafter washed. During the last washing or in a last separate step before the peroxide addition, magnesium is added in an amount of 0.1-10 kg magnesium per ton of pulp, preferably more than 2 kg per ton of pulp.

US-A-4 915 785 discloses a single stage process for the bleaching of high yield lignocellulose pulp (mechanical pulp) to enhance brightness levels with hydrogen peroxide in the presence of magnesium sulfite and sodium silicate with a substantial reduction in the wasteful, non-bleaching reactions of hydrogen peroxide. None of these references teaches to use high molecular weight silicates for improving the brightening properties of the pulp.

EP-B-0 677 124 discloses a process for chlorine-bleaching of a chemical pulp, which process is characterized in that the peroxide bleaching is effected at a temperature exceeding 90°C and at a pressure in the bleaching vessel which exceeds 2 bar and in that the cross-sectional area of the bleaching vessel exceeds 3 m², and in that the area of the metal surface expose towards the interia of the bleaching vessel is less than 4 Vm², wherein V indicates the volume of the vessel in m².

### SUMMARY OF THE INVENTION

The present invention provides a combination of additives and methods for brightening pulps containing less than 18% lignin. The invention can be used in either the peroxide, oxygen, or peroxide/oxygen brightening stages. The additives according to the present invention include an aqueous sodium silicate solution, an alkali agent, and a magnesium compound which dissociates in the solution to form Mg(OH)⁺ cations. The alkali agent is added in an amount sufficient to maintain a pH of at least about 8, and the magnesium compound is added in an amount to achieve, along with any other dissociated magnesium, an Mg:SiO₂ mass ratio of between about 1:15 to about 1:2. At least 25% of the silicates have a molecular weight of at least 10.000 Dalton.

A method for brightening pulp according to the present invention involves mixing pulp containing less than 18% lignin with an aqueous sodium silicate solution, an alkali agent, and a magnesium compound which dissociates in the solution to form Mg(OH)⁺ cations. The alkali agent and magnesium compound are added to achieve the same pH range and weight ratio mentioned above. The method also includes heating the mixture to allow the mixture to react to cause a portion of the lignin in the pulp to degrade.

According to another embodiment of the present invention directed to the peroxide or peroxide/oxygen brightening stages, a method for brightening pulp containing transition metals, hydrogen peroxide, and less than 18% lignin includes first forming a sodium silicate mixture having a high percentage of high molecular weight silicates. This is accomplished by mixing sodium silicate and a magnesium compound which dissociates in the solution to form Mg(OH)⁺ cations. This sodium silicate mixture is then added to the pulp to adsorb at least a portion of the transition metals.

The present invention also includes an aqueous composition for use in brightening pulps. The composition includes pulp containing less than 18% lignin, an aqueous sodium silicate solution, an alkali agent, and a magnesium compound which dissociates in the solution to form Mg(OH)⁺ cations. The alkali agent and magnesium compound are added to achieve the same pH range and weight ratio mentioned above.

It is to be understood that both the foregoing general description and the following detailed description are exemplary, but are not restrictive, of the invention.

### DETAILED DESCRIPTION OF THE INVENTION

The present invention is directed to the brightening of certain pulps during peroxide, oxygen, or peroxide/oxygen brightening. As used herein, the term "brightening stage" shall mean either a peroxide stage, an oxygen stage, or a peroxide/oxygen stage. The typical operating conditions and conventional additives to these stages are well known. During such brightening, hydrogen peroxide serves to degrade carbonyl groups of lignin, rendering them more water soluble. In the absence of such degradation, lignin would remain in the pulp, causing the brightness of the pulp to remain lower than would be if such lignin were removed. Transition metals present in the pulp undesirably react with hydrogen peroxide thereby precluding hydrogen peroxide from serving its function of degrading lignin. The present invention is based in part on the recognition that higher molecular weight silicates assist in adsorbing transition metals thus preventing them from undesirably reacting with hydrogen peroxide. The present invention is also based on the recognition that Mg(OH)⁺ plays a significant role in the molecular weight distribution of a sodium silicate solution. More particularly, the presence of Mg(OH)⁺ in a sodium silicate solution, over a certain Mg:SiO₂ mass ratio, enhances the formation of higher molecular weight silicates.

Accordingly, the present invention is directed to various compositions and methods embodying this concept. The invention provides a combination of additives (either to hydrogen peroxide, oxygen, or a combination thereof, depending on which one of the three brightening stages is being employed) for brightening pulps containing less than 18% lignin. In this case, these additives include an aqueous sodium silicate solution, an alkali agent, and a magnesium compound which dissociates in the solution to form Mg(OH)⁺ cations. The invention also encompasses an aqueous composition for use in brightening pulps comprising pulp containing less than 18 % lignin, hydrogen peroxide (either as an additive or as reacted from reaction [6] above), an aqueous sodium silicate solution, an alkali agent, and a magnesium compound which dissociates in the solution to form Mg(OH)⁺ cations. The present invention also provides a method for brightening pulp including forming a mixture of the pulp, hydrogen peroxide, aqueous sodium silicate solution, alkali agent, and magnesium compound, then heating the mixture to allow it to react to cause a portion of the lignin to degrade. Finally, the invention is characterized as a method for brightening pulp containing transition metals and less than 18% lignin. This method includes the steps of forming a sodium silicate mixture having a high percentage of high molecular weight silicates by mixing sodium silicate and a suitable magnesium compound, and adding the sodium silicate mixture to the pulp.

The pulp used in connection with the present invention is defined broadly as any pulp having less than 18% lignin (on pulp). Unless otherwise specified, all percentages of lignin include all forms of lignin and are given as weight percentages of the total pulp, on a dry weight basis, so that 18 % lignin means that there are 18 grams of lignin in a 100 gram sample of pulp (excluding the weight of water).

Stated another way, the invention can be used with any pulp in which more than 50 % of the lignin (by weight, on wood) is removed during pulping. This means that more than half of the original lignin present in the wood is removed during the pulping process. For softwoods, having an average lignin content of 28.6% (by weight, on wood), the removal of half of the original lignin content of the wood during a conventional chemical pulping process results in a pulp having 23.3% lignin (on pulp). For hardwoods, having an average lignin content of 24.1 % (by weight, on wood), the removal of half of the original lignin content of the wood during a conventional chemical pulping process results in a pulp having 18.0% lignin (on pulp). The development of these final lignin contents factors in the yield from conventional chemical pulping processes. Thus, any pulp with less than 18 % lignin (on pulp) would typically include at least some pulp which was processed by chemical pulping or was derived from a wood having a relatively low initial content of lignin.

In general, chemical pulping processes are continued until the lignin content is reduced to about 5% (on pulp) or less. It is preferable to use the present invention to brighten such pulps. In addition, chemical pulps typically undergo further delignification before the final brightening stage (i.e., peroxide or peroxide/oxygen) such that the pulps contain about 1-2% lignin before the final brightening stage. Pulps brightened by the present invention can also include such pulps which have been further delignified. The present invention can also be used to brighten pulps having recycled pulps, in which chemical and mechanical pulps are mixed, as long as the average lignin content is less than about 18%. Pulps brightened by the present invention also include semichemical pulps with lignin content varying from approximately 10 to 18%. In Example 4 below, bleached and unbleached samples of de-inked mixed office waste consisting of 65% sorted white ledger and 35% office pack were obtained from a mill in the American Midwest.

The additives of the present invention are used in the peroxide, oxygen, or peroxide/oxygen stages of brightening. The process parameters of these stages are well known. For example, a typical charge of peroxide loading is 20 kg of hydrogen peroxide per metric ton of pulp. The hydrogen peroxide is mixed while the mixture is heated, typically to a temperature of between about 90°C to about 130°C, often 110°C. Water is also added, typically to achieve a consistency of about 15% solids. Of course, reaction time, temperature, and consistency are all interrelated and can be varied in a known manner. A hydrogen peroxide/oxygen stage is similar to a hydrogen peroxide stage except that the slurry is pressurized with oxygen.

An oxygen stage is similar to a hydrogen peroxide/oxygen stage except that no hydrogen peroxide is added. Oxygen delignification is also conducted over a wider consistency range (10 % to 35% solids) but 12% to 15% solids is typical. In general, an oxygen stage does not brighten as well as a peroxide stage or as a peroxide/oxygen stage. Oxygen or an oxygen-containmg gas (such as air) can be used to pressurize the mixture, and the partial pressure of oxygen typically ranges between 0.38 MPa and 1.48 MPa.

An additive of the present invention is an aqueous sodium silicate solution. Any commercially available aqueous sodium silicate solution may be used, although it is preferable to use as pure of a sodium silicate solution as is practically possible. The sodium silicate solution may be added in an amount to achieve a concentration of from about 0.14% to about 1.4% SiO₂ on pulp. Preferably, the sodium silicate solution is added in an amount to achieve a concentration of from about 0.28% to about 1.12% SiO₂ on pulp.

Another additive according to the present invention is a magnesium compound which dissociates in the solution to form Mg(OH)⁺ cations. The magnesium compound should be added in an amount to achieve, along with any other dissociated magnesium, an Mg:SiO₂ mass ratio of between about 1:15 to about 1:2. Preferably, the Mg:SiO₂ mass ratio is between about 1:15 to about 1:3. Most preferably, the Mg:SiO₂ mass ratio is between about 1:10 to about 1:3. The mass ratio is of the total magnesium available for formation into Mg(OH)⁺, including any of the magnesium added and any magnesium inherent in the pulp and existing in a form which readily dissociates and forms Mg(OH)⁺ over a pH range of at least 8:

The magnesium compound is added in an amount to achieve an actual concentration of from about 0.01 % to about 0.2 % Mg on pulp (again including any other source of available magnesium). More preferably, the magnesium compound is added in an amount to achieve a concentration of from about 0.02% to about 0.2% Mg on pulp. Preferably, the magnesium compound is magnesium sulfate, added as MgSO₄ or MgSO₄·7H₂O. Alternatively, the magnesium compound is MgO, MgCl₂, Mg(OH)₂ and/or MgNO₃, among others. Any number of magnesium compounds can be used, as long as they readily form Mg(OH)⁺ at pH values of at least 8 and are not detrimental to process equipment.

A critical step in the present invention is the formation of the hydrolyzed magnesium cation Mg(OH)⁺. It is believed that this cation neutralizes dissociated silanol groups and causes silicate polymerization, as summarized by the equations written below:

Another additive of the present invention is an alkali agent added in an amount sufficient to maintain a pH of the solution of at least about 8. At pH values of at least about 8, magnesium exists as Mg(OH)⁺ in an amount sufficient to initiate reaction [9] above. More preferably, the alkali agent is selected and added in an amount sufficient to maintain the pH to a range of between 8 and 12. The alkali agent may be NaOH, Na₂O, MgO, Mg(OH)₂, K₂O, KOH, CaO, and/or Ca(OH)₂. Preferably, the non-calcium containing compounds are selected to minimize the formation of silicate scales. Such silicate scales can be detrimental to the quality of the paper product and must be removed periodically resulting in costly stoppages of the process. Because MgO and Mg(OH)₂ can serve two functions, namely that as the magnesium compound which readily forms Mg(OH)⁺ and as an alkali agent, then the magnesium compound and alkali agent can be combined as one additive in some cases.

According to a method of the present invention, the pulp is brightened by mixing the pulp with hydrogen peroxide, an aqueous sodium silicate solution, an alkali agent added in an amount sufficient to maintain the pH of the solution at least about 8, and a magnesium compound which dissociates in the solution to form Mg(OH)⁺ cations, wherein the magnesium compound is added in an amount to achieve, along with any other dissociated magnesium, an Mg:SiO₂ mass ratio of between about 1:15 to about 1:3. This mixture is then heated, which allows the mixture to react to cause a portion of the lignin to degrade (i.e., to break down into a more soluble form to be washed away). In the case where a hydrogen peroxide/oxygen stage is used, the mixture is also pressurized with oxygen, in a known manner. While continuously heated, the chemicals are mixed into the pulp slurry which is retained at an elevated temperature for a period of time sufficient to allow the degradation reactions of the lignin to occur. This typically is between 30 minutes and four hours, depending on the temperature and concentration of the additives in the pulp. Typically, the mixture is heated to a temperature of between about 90°C and about 130°C.

As mentioned above, the present invention relies on the formation of high molecular weight silicates to adsorb transition metals to avoid the decomposition of hydrogen peroxide by transition metals. Accordingly, the present invention can be characterized as a method for brightening pulp by forming a sodium silicate solution having a high percentage of high molecular weight silicates by mixing sodium silicate and a magnesium compound which dissociates in the solution to form Mg(OH)⁺ cations. Then, the sodium silicate solution is added to the pulp to adsorb at least a portion of the transition metals of the pulp. Any increased amount of higher molecular weight silicates appears to improve the adsorption of transition metals, and the constituents are added such that the sodium silicate solution has at least 25% of the silicates with a molecular weight of at least 10,000 daltons.

It is not believed that the order of addition is important to the functioning of the present invention. Typically, the magnesium compound is Epsom salt (MgSO₄·7H₂O) and is either first dissolved in water or dissolved directly in a commercial aqueous sodium silicate solution. Then the alkali agent(s) is added followed by H₂O₂. The combination is then mixed into the pulp slurry.

### EXAMPLES

The following examples are included to more clearly demonstrate the overall nature of the invention. These examples are exemplary, not restrictive, of the invention.

### Example 1

A kraft pulp was delignified by the ODEop partial sequence and had a kappa number of 2.7 and a viscosity of 19.0 cp. The ODEop partial sequence is called elemental chlorine-free or ECF. The pulp had a low initial Mg content (< 50 ppm). The pulp was P/O (P=H₂O₂; O=O₂) bleached at 12% consistency and 110°C for 2 hours using reagent grade H₂O₂, NaOH and MgSO₄·7H₂O. A technical grade sodium silicate solution sold by Fisher Scientific, which contained some transition metals, was used. An H₂O₂ charge of 1.5% by weight on pulp was used with 2.0-2.3% NaOH by weight on pulp. The initial O₂ pressure for all P/O experiments was 0.38 MPa.

A first series of experiments was run to determine the effect of magnesium sulfate addition on the brightening of this ECF pulp. Table 1 shows both percentage of the constituents in each sample added to the pulp (on a dry weight basis) and the brightness, yield, viscosity, and residual H₂O₂. Samples 1 through 4 have the same amount of silicate, sodium hydroxide, and hydrogen peroxide, while the amount of the magnesium compound (in this case, magnesium sulfate) increases from Samples 1 through 4. In all of the tables in the examples, "silicate" refers to the weight percent of a 41 Bé silicate solution (28.7% SiO₂) that was added. For all examples, the brightness was determined in accordance with TAPPI Standard T452 om-92. In addition, the pulp yield is the mass of washed pulp from the P or P/O stage divided by the mass of the feed to the stage. The viscosity and residual hydrogen peroxide (given as a percentage of the initial dose) were determined by known methods, including TAPPI Standard T230 om-94 for viscosity and iodometric titration for residual H₂O₂.

**Table 1**

| Effect of Magnesium Sulfate Application on P/O Bleaching of First ECF Kraft Pulp | | | | |
|---|---|---|---|---|
| | Sample 1 | Sample 2* | Sample 3* | Sample 4 |
| Silicate, % on pulp | 4.0 | 4.0 | 4.0 | 4.0 |
| NaOH, % on pulp | 2.3 | 2.3 | 2.3 | 2.3 |
| H₂O₂, % on pulp | 1.5 | 1.5 | 1.5 | 1.5 |
| MgSO₄·7H₂O % on pulp | 0.0 | 0.25 | 0.5 | 0.75 |
| SiO₂, % on pulp | 1.148 | 1.148 | 1.148 | 1.148 |
| Mg, % on pulp | 0.0 | 0.025 | 0.050 | 0.075 |
| Mg:SiO₂ mass ratio | 0 | 1:46 | 1:23 | 1:15 |
| End pH | 10.2 | 10.5 | 11.0 | 11.2 |
| | | | | |
| Brightness, % | 79.8 | 84.0 | 84.2 | 85.3 |
| Yield, % | 97.2 | 97.7 | 98.1 | 98.2 |
| Viscosity, cp | 8.8 | 11.4 | 13.5 | 14.1 |
| | | | | |
| Residual H₂O₂, % | | | | |
| 30 Minutes | 2 | 25 | 35 | 33 |
| 60 Minutes | 0 | 15 | 22 | 30 |
| 120 Minutes | 0 | 2 | 7 | 10 |

| | | | | |
|---|---|---|---|---|
| * not claimed | | | | |

Table 1 shows that an MgSO₄·7H₂O charge of 0.25% on pulp (250 ppm Mg on pulp) increased brightness significantly, namely from 79. 8 % to 84.0 %. Also, the brightness increased further when 0.50 and 0.75% MgSO₄ 7H₂O was used. The interesting and totally novel result from Table 1 is the increase in pulp yield caused by the addition of magnesium sulfate. Kraft pulps can be dissolved in a solution of cupriethylenedianine, and the viscosity of the solution is an indicator of the degree of polymerization of the cellulose in the pulp. It can be seen that a higher charge of magnesium sulfate also resulted in higher viscosities (less depolymerization of cellulose during H₂O₂ brightening). However, the lowest viscosity (no MgSO₄·7H₂O) corresponds to an average DP of 815. It is unlikely that cellulose molecules of such high DP would solubilize. Therefore, it appears that hemicelluloses were being dissolved. Most likely, the free radicals from H₂O₂ decomposition were causing depolymerization of the hemicelluloses to a degree that resulted in their solubilization.

### Example 2

A second ECF pulp sample was obtained from the same mill serving as the source of the pulp used in Example 1. It had a kappa number of 2.4 and a viscosity of 20.5 cp. The transition metal content of the first ECF pulp was not measured but the second pulp contained 6 ppm Mn, 8 ppm Fe, and 2 ppm Cu. These values were lowered to 0.3, 3.7 and 1.5 ppm, respectively, after treatment with Na₅DTPA. Sample 2 was bleached at 100°C, while Samples 1, 3, and 4 were bleached at 110°. Table 2 varies the charge of sodium silicate, with Samples 1 and 2 having no silicate added, while Samples 3 and 4 have a 2.0 and 4.0 % charge, respectively.

**Table 2**

| Effect of Silicate on P/O Bleaching of Second ECF Kraft Pulp. Chelated Pulp: 0.3 ppm Mn, 3.7 ppm Fe and 1.5 ppm Cu | | | | |
|---|---|---|---|---|
| | Sample 1 ^{x} | Sample 2 ^{x} | Sample 3 | Sample 4 ^{x} |
| Silicate, % on pulp | 0.0 | 0.0 | 2.0 | 4.0 |
| NaOH, % on pulp | 2.0 | 2.0 | 2.0 | 2.0 |
| H₂O₂, % on pulp | 1.5 | 1.5 | 1.5 | 1.5 |
| MgSO₄ · 7H₂O% on pulp | 0.5 | 0.5 | 1.0 | 0.5 |
| SiO₂, % on pulp | 0.0 | 0.0 | 0.574 | 1.148 |
| Mg, % on pulp | 0.05 | 0.05 | 0.10 | 0.05 |
| Mg:SiO₂ mass ratio | NA* | NA* | 1:6 | 1:23 |
| End pH | 10.9 | 10.9 | 10.5 | 10.9 |
| | | | | |
| Brightness, % | 85.1 | 84.3 | 85.7 | 85.3 |
| Yield, % | 98.0 | 98.3 | 98.2 | 98.6 |
| Viscosity, cp | 12.6 | 13.7 | 16.3 | 13.7 |
| | | | | |
| Residual H₂O₂, % | | | | |
| 30 Minutes | 24.9 | 31.5 | 38.2 | 41.5 |
| 60 Minutes | 10.0 | 19.9 | 28.2 | 31.5 |
| 120 Minutes | 3.3 | 6.6 | 14.9 | 14.9 |

| | | | | |
|---|---|---|---|---|
| *Not applicable | | | | |
| ^{x} not claimed | | | | |

Table 2 shows slight increases in brightness and yield of the chelated sample when the amount of sodium silicate is increased. The low transition metal contents of this pulp, particularly the 0.3 ppm Mn, can be achieved in only a few commercial installations. More significantly, the presence of sodium silicate shows a significant increase in residual hydrogen peroxide, which is important in maintaining brightness. In the absence of silicate, the H₂O₂ residual for most pulp samples would be zero after two hours at 110°C.

### Example 3

Four more samples of the same ECF pulp used in Example 2, having a kappa number of 2.4 and a viscosity of 20.5 cp, were tested. In this case, the pulp was unchelated. In Samples 1 and 2 below, the temperature of the stage was 90°C while the temperature of Samples 3 and 4 was 110°C. Samples 1 and 3 contained no silicate, while Samples 2 and 4 did.

**Table 3**

| Effect of Temperature on P/O Bleaching of Second ECF Kraft Pulp. Unchelated Pulp: 6 ppm Mn, 8 ppm Fe and 2 ppm Cu | | | | |
|---|---|---|---|---|
| | Sample 1 ^{x} | Sample 2 | Sample 3 ^{x} | Sample 4 |
| Temperature, °C | 90 | 90 | 110 | 110 |
| Silicate, % on pulp | 0 | 2.0 | 0 | 2.0 |
| NaOH, % on pulp | 2.0 | 2.0 | 2.0 | 2.0 |
| H₂O₂, % on pulp | 1.5 | 1.5 | 1.5 | 1.5 |
| MgSO₄ · 7H₂O% on pulp | 0.5 | 1.0 | 0.5 | 1.0 |
| SiO₂, % on pulp | 0.0 | 0.574 | 0.0 | 0.574 |
| Mg, % on pulp | 0.05 | 0.1 | 0.05 | 0.1 |
| Mg:SiO₂ mass ratio | NA | 1:6 | NA | 1:6 |
| End pH | 11.3 | 11.6 | 9.9 | 10.9 |
| | | | | |
| Brightness, % | 78.0 | 79.9 | 79.7 | 81.8 |
| Yield, % | 98.5 | 98.7 | 97.9 | 98.5 |
| Viscosity, cp | 15.4 | 15.7 | 11.5 | 14.1 |
| | | | | |
| Residual H₂O₂, % | | | | |
| 30 Minutes | 3.3 | 18.2 | 1.7 | 10.0 |
| 60 Minutes | 1.7 | 10.0 | 0.0 | 5.0 |
| 120 Minutes | 0.0 | 5.0 | 0.0 | 3.3 |

| | | | | |
|---|---|---|---|---|
| ^{x} not claimed | | | | |

Table 3 shows that, at either temperature, the inclusion of sodium silicate improves the brightening process. At 90°C, a sample having sodium silicate gave no noticeable improvement in yield but 1.9% increase in brightness. At 110°C, a sample including sodium silicate caused a 0.6% increase in yield and a 2.1 % increase in brightness. Also, as before, the presence of sodium silicate showed a significant increase in residual hydrogen peroxide, which is important in maintaining brightness.

### Example 4 (Comparison)

Bleached and unbleached samples of de-inked, mixed office waste (MOW) consisting of 65% sorted white ledger and 35% office pack were obtained from a mill in the American Midwest. This pulp sample was from almost exclusively chemical pulps. The properties of the samples are summarized in Table 4. High positive b* value indicates a yellowish tint and a high negative value indicates a bluish tint. A high positive a* value indicates a reddish tint and a high negative value indicates a greenish tint. The aim of bleaching is to decrease the absolute a* and b* values to as close to zero and increase the L* value as high as possible. As shown in Table 4, the effect of the addition of silicate and magnesium sulfate to MOW was determined.

**Table 4**

| Effect of Silicate Addition on P/O Bleaching of Mixed Office Waste (MOW) | | | | |
|---|---|---|---|---|
| Pulp¹ | MOW | MOW | BL. MOW | BL. MOW |
| Silicate, % on pulp | 0.0 | 4.0 | 0.0 | 4.0 |
| NaOH, % on pulp | 2.3 | 2.3 | 2.3 | 2.3 |
| H₂O₂, % on pulp | 1.5 | 1.5 | 1.5 | 1.5 |
| MgSO₄·7H₂O on pulp | 0.5 | 0.5 | 0.5 | 0.5 |
| SiO₂, % on pulp | 0.0 | 1.148 | 0.0 | 1.148 |
| Mg, % on pulp | 0.05 | 0.05 | 0.05 | 0.05 |
| Mg:SiO₂ mass ratio | NA | 1:23 | NA | 1:23 |
| End pH | 10.1 | 10.2 | 10.0 | 10.0 |
| Brightness, % | 77.9 | 80.4 | 85.4 | 88.3 |
| | | | | |
| L* | 91.51 | 91.86 | 94.79 | 95.24 |
| a* | -0.46 | 0.22 | 0.27 | -0.07 |
| b* | 1.67 | 0.73 | 1.68 | 0.48 |
| Yield, % | 95.4 | 96.5 | 97.3 | 97.4 |
| Viscosity, cp | 9.8 | 11.0 | 9.7 | 11.1 |

| Residual H₂O₂, % of Applied | | | | |
|---|---|---|---|---|
| 30 Minutes | 2 | 27 | 3 | 28 |
| 60 Minutes | 0 | 10 | 1 | 15 |
| 120 Minutes | 0 | 5 | 0 | 7 |

| | | | | |
|---|---|---|---|---|
| ¹Mixed office waste (MOW) pretreated with 0.2% DTPA: Brightness, 74.2; L*=89.78; a*=0.76; b*=1.77. Commercially bleached mixed office waste (BLMOW) pretreated with 0.2% DTPA: Brightness, 83.6, L*=94.4; a*=0.28; b*=1.72. | | | | |

It can be seen (footnotes of Table 4) that H₂O₂ bleaching in the mill (∼ 1.0% H₂O₂, ∼ 95°C) did not significantly lower the b* value. Both the unbleached and commercially bleached samples were treated with Na₅DTPA then brightened with 1.5% H₂O₂ at 110°C. For the unbleached sample, the inclusion of 4.0% silicate resulted in an improvement of 2.5 brightness points. The a* and b* values were closer to zero as well. Similar benefits were obtained when the commercially bleached pulp was brightened further. Without silicate, no significant decrease in b* was obtained. A high temperature and high H₂O₂ residuals apparently are required to destroy the colored contaminants responsible for the b* value. The inclusion of silicate increased the yield of the unbleached pulp by 1.1%.

### Example 5

The results in Table 1 showed increased brightness with an increase in the dose ratio of MgSO₄·7H₂O:sodium silicate (41 Bé). The dose ratio was increased further in Table 2 where 2% sodium silicate and 1.0% MgSO₄·7H₂O on pulp were used (i.e., Sample 3 of Table 2), which resulted in the highest brightness (85.7%) for the ECF pulps. In this Example, the effect of dose ratio on the brightening of a totally chlorine-free (TCF) pulp is investigated.

The TCF pulp (kraft) was from a Swedish mill and it had a kappa number of 7.4 and a viscosity of 23.4 cp. It also contained 1.9 ppm Mn, 4.7 ppm Fe, and 0.8 ppm Cu. After it was acid-washed it contained 0.1 ppm Mn, 4.0 ppm Fe, and 0.8 ppm Cu. The acid-washed pulp was brightened with various dose ratios of MgSO₄ 7H₂O:sodium silicate. The H₂O₂ and NaOH charges were 2.0% and 2.5 % on pulp, respectively, and the pulps were brightened for two hours at 110°C and 12% consistency.

**Table 5**

| Effect of Silicate and MgSO₄ · 7H₂O on P/O Bleaching of Acid-Washed TCF Pulps | | | | |
|---|---|---|---|---|
| | Sample 1 | Sample 2 | Sample 3 | Sample 4 |
| Silicate, % on pulp | 0 | 4.0 | 2.0 | 1.0 |
| NaOH, % on pulp | 2.5 | 2.5 | 2.5 | 2.5 |
| H₂O₂, % on pulp | 2.0 | 2.0 | 2.0 | 2.0 |

| | Sample 1 ^{x} | Sample 2 ^{x} | Sample 3 | Sample 4 |
|---|---|---|---|---|
| MgSO₄·7H₂O% on pulp | 0.5 | 0.5 | 1.0 | 1.0 |
| SiO₂, % on pulp | 0 | 1.148 | 0.574 | 0.287 |
| Mg, % on pulp | 0.05 | 0.05 | 0.10 | 0.10 |
| Mg:SiO₂ mass ratio | NA | 1:23 | 1:6 | 1:3 |
| End pH | 10.5 | 11.3 | 10.9 | 10.8 |
| | | | | |
| Brightness, % | 75.4 | 78.2 | 79.4 | 77.9 |
| Yield, % | 96.3 | 98.2 | 98.3 | 98.0 |
| Viscosity, cp | 9.1 | 13.1 | 15.5 | 12.8 |
| | | | | |
| Residual H₂O₂, % | | | | |
| 30 Minutes | 15 | 32 | 37 | 31 |
| 60 Minutes | 4 | 19 | 16 | 8 |
| 120 Minutes | 0 | 5 | 5 | 1 |

| | | | | |
|---|---|---|---|---|
| ^{x} not claimed | | | | |

The brightness and yield were relatively low when silicate was excluded (Sample 1 of Table 5). The highest brightness was obtained with MgSO₄·7H₂O:sodium silicate dose ratio of 1%:2%. The next highest brightness was for dose ratio 0.5%:4%, followed by 1%:1%.

A general trend from the first five tables is that, for a given temperature, higher brightness and yields are obtained as H₂O₂ stabilization is improved (higher residuals). There is not an exact correlation because, for these experiments, the accuracy on H₂O₂ residual was about ±5% of the initial charge. However, final brightness in Table 5 correlates with H₂O₂ residual after 30 minutes.

The three dose ratios in Table 5, i.e. 0.5:4.0; 1.0:2.0; and 1.0;1.0, were used in a pulp-free system to deactivate 1 ppm, each Mn²⁺, Fe³⁺, and Cu²⁺ added simultaneously to the alkaline solution. For each dose ratio, the initial solution phase concentrations of H₂O₂, MgSO₄ ·7H₂O, and sodium silicate were identical to when pulp was present. In the absence of pulp, less NaOH was required to achieve pH 11.2 taken as a rough average for P/O bleaching. The solutions were retained at 110°C for two hours then cooled and ultra-filtration was used to separate high and low molecular weight silicates. Membranes with 10,000 MW cutoff were used.

The results will be analyzed in terms of ppm Si in solution. The 41 Bé silicate solution that was used contained 28.7% SiO₂. Therefore 4% silicate on pulp corresponds to 1.148 SiO₂ on pulp or 0.536 % Si on pulp. One hundred grams of pulp at 12% consistency is associated with 733 mL of solution (assuming a specific gravity of 1.0). Therefore, the Si concentration is 0.536 g in 733 mL or 0.731 g/L (∼730 ppm). The solutions passing through the membrane were analyzed for Si, Mn, Fe and Cu concentrations by ICP spectroscopy. The results are presented in Table 6.

**Table 6**

| Mg and Silicate Conc., ppm in Solution | Conc. Passing Through Membrane | | | |
|---|---|---|---|---|
| | Si | Mn | Fe | Cu |
| 68 ppm Mg* + 730 ppm Si | 617 | 0.008 | 0.023 | 0.027 |
| 136 ppm Mg + 365 ppm Si | 194 | 0.001 | 0.001 | 0.016 |
| 136 ppm Mg + 183 ppm Si | 56 | 0.004 | 0.001 | 0.018 |

| | | | | |
|---|---|---|---|---|
| *0.5 % MgSO₄ · 7H₂O on pulp | | | | |

Table 6 shows that in the case of 0.5 % MgSO₄·7H₂O and 4% silicate, 85 % of the Si passes through the membrane as low molecular weight compounds. However, less than 3% of the Fe and Cu and less than 1 % of the Mn pass through. The transition metals appear to be bound to the high molecular weight silicate retained on the membrane. The data would suggest that 1.0 % MgSO₄·7H₂O and 2.0 % silicate give the best transition metal deactivation, particularly of Mn which is believed to be the most aggressive catalyst for H₂O₂ decomposition. The significance of the differences between 1, 4, and 8 ppb Mn or 16, 18 and 27 ppb Cu in solution might be deemed insignificant. However, there is no doubt that it is the high molecular weight silicate that adsorbs or complexes the transition metals. The amount of high molecular weight silicate (greater than 10,000 daltons) for the various formulations are 113 ppm Si for 0.5%:4.0%; 127 ppm for 1.0%:1.0%; and 171 ppm for 1.0%:2.0%. The clear superiority of the 1%:2.0% formulation in Table 6 is now evident.

### Example 6

The ECF pulp of Example 1 used for peroxide/oxygen bleaching was treated with an acidic chlorine dioxide stage while the TCF pulp was acid-washed. Calcium that was bound to the pulps dissolved in the acidic solutions and was washed out. Six effluents from peroxide/oxygen bleaching of ECF pulps and five effluents from TCF pulps were collected and divided in two. Calcium chloride was added to one half of each effluent to give a concentration of 50 ppm Ca²⁺ in solution. Smaller volumes of the straight and calcium-enriched effluents were adjusted to pH values of 9.0 and 10.0, than one inch square strips (1 inch = 2.54cm) of 20-mesh stainless steel were placed in each solution or slurry. All of the selected effluents contained both epsom salt and sodium silicate. There was no magnesium silicate precipitate at either pH value, but there were calcium-magnesium silicate precipitates in most of the eleven effluents that were enriched with calcium chloride.

Each metal strip weighed about 1.6 grams initially and, surprisingly, none of them gained any weight when placed in any of the magnesium silicate solutions or the calcium-magnesium silicate slurries for more than 96 hours at room temperature (about 20°C). When taken from the solution or slurry, each strip weighed within 2 milligrams of its initial weight after washing and airdrying. This confirms that calcium silicates adhere to metals while calcium-magnesium and magnesium silicates do not.

Unbleached pulps are normally not acid-washed or treated with chelating-agents before O₂ delignification. Therefore, pulps normally enter an oxygen delignification stage with higher concentrations of calcium than that of pulps entering a peroxide/oxygen stage. However, if 1 % epsom salt and 2% sodium silicate is added, there would be enough magnesium cations to chemisorb most of the dissociated silanol groups at pH values less than 11. Since magnesium cations are preferentially chemisorbed over calcium cations, any potential precipitate would be rich in magnesium. It is unlikely that such precipitates would scale the oxygen washers, where the pulp is washed after oxygen delignification. Scaling is unlikely at the high pH values of the black liquor (i.e., washed liquor from the unbleached pulp) evaporators, which are used to evaporate moisture after washing and before burning the now concentrated black liquor in a kraft recovery furnace. The likely scenario is that the calcium-magnesium silicate will pass through the kraft recovery furnace and be removed with the dregs at the green liquor clarifier. (Green liquor is the viscous fluid removed from the bottom of the recovery furnace and is made up primarily of inorganic compounds, such as sodium sulfide and sodium carbonate.) After removal, green liquor is diluted and insoluble materials (i.e., dregs) are separated by sedimentation. A high rate of sedimentation is observed for these calcium-magnesium silicate particles.

The effect of the magnesium sulfate/sodium silicate combination on oxygen delignification is demonstrated below in Table 7. Two-stage oxygen delignification of a 41 kappa number kraft pulp was simulated by adding 2% NaOH on pulp and 0.72 MPa of oxygen at 12% consistency and 90°C for 30 minutes, followed by a second NaOH injection (1.0% NaOH on pulp), restoration of oxygen pressure, and 30 minutes of additional retention. The standard oxygen included 0.5% epsom salt on pulp added during the preheat stage, i.e., before all other chemicals. When silicate was used, 1% Epsom salt on pulp was added at the preheat stage and 2 % sodium silicate was added along with the first sodium hydroxide injection. Silicate additions significantly improved delignification selectivity (kappa number versus viscosity). Pulp brightness is also increased.

**Table 7**

| Effect of Silicate Addition on Kappa Number and Viscosity After O₂ Delignification | | |
|---|---|---|
| | Standard Oxygen | O₂ with Silicate |
| MgSO4 7H₂O, % on pulp | 0.5 | 1.0 |
| Silicate, % on pulp | 0 | 2.0 |
| end pH | 11.0 | 11.6 |
| Brightness, % | 28.2 | 30.8 |
| Kappa No. | 20.4 | 20.0 |
| Viscosity, cP | 21.2 | 24.7 |
| ¹Laboratory pulp made from 5 kg of chips, kappa number 41, viscosity 35 cP and screened yield of 47.8% | | |

The improvement in viscosity is significant because viscosity is lowered further by most delignification and brightening stages, including P/O stages. If the viscosity is lowered below 10-12 cP (DP ∼ 1000) then the strength values of paper made from the pulp decline dramatically.

Although illustrated and described herein with reference to certain specific embodiments and examples, the present invention is nevertheless not intended to be limited to the details shown. Rather, the claims should be read to include various modifications within the scope and range of equivalents of the claims, without departing from the spirit of the invention.

## Claims

1. A combination of additives for use in a brightening stage of pulps containing less than 18 % lignin, said combination comprising: an aqueous sodium silicate solution; an alkali agent added in an amount sufficient to maintain a pH of said solution at least about 8; and a magnesium compound which dissociates in said solution to form Mg(OH)⁺ cations, wherein said magnesium compound is added in an amount to achieve, along with any other dissociated magnesium, an Mg:SiO₂ mass ratio of between about 1:15 to about 1:2, and wherein at least 25 % of the silicates have a molecular weight of at least 10,000 Daltons.

2. A combination of additives in accordance with claim 1, wherein said Mg:SiO₂ mass ratio is between about 1:15 to about 1:3.

3. A combination of additives in accordance with claim 1, wherein said alkali agent is added in an amount sufficient to maintain the pH of said solution within the range of from about 8 to about 12.

4. A combination of additives in accordance with claim 1, wherein said magnesium compound is magnesium sulfate, added as MgSO₄ or MgSO₄·7H₂O.

5. A combination of additives in accordance with claim 1, wherein:
said aqueous sodium silicate solution is added in an amount to achieve a concentration of from about 0.14 % to about 1.4 % SiO₂ on pulp; and
said magnesium compound is added in an amount to achieve a concentration of from about 0.01 % to about 0.2 % Mg on pulp.

6. A combination of additives in accordance with claim 5, wherein:
said aqueous sodium silicate solution is added in an amount to achieve a concentration of from about 0.28 % to about 1.12 % SiO₂ on pulp; and
said magnesium compound is added in an amount to achieve a concentration of from about 0.02 % to about 0.2 % Mg on pulp.

7. A combination of additives in accordance with claim 1, wherein said alkali agent is selected from the group consisting of at least one of NaOH, Na₂O, MgO, Mg(OH)₂, K₂O, KOH, CaO, and Ca(OH)₂.

8. A combination of additives in accordance with claim 1, wherein said magnesium compound is selected from the group consisting of at least one of MgO, MgCl₂, Mg(OH)₂ and MgNO₃.

9. A combination of additives in accordance with claim 1 further comprising hydrogen peroxide.

10. Use of a combination according to one of claims 1 to 9 in a brightening stage of pulps containing less than 18 % lignin.

11. The use of claim 10, wherein said pulp contains less than 5 % lignin.

12. The use of claim 11, wherein said pulp contains less than 2 % lignin.

13. A method for brightening pulp comprising the steps of:
mixing pulp containing less than 18 % lignin with hydrogen peroxide, an aqueous sodium silicate solution; an alkali agent added in an amount sufficient to maintain the pH of said solution at least about 8; and a magnesium compound which dissociates in said solution to form Mg(OH)⁺ cations, wherein said magnesium compound is added in an amount to achieve, along with any other dissociated magnesium, an Mg:SiO₂ mass ratio of between about 1:15 to about 1:2, to form a mixture; and wherein at least 25 % of the silicates have a molecular weight of at least 10,000 Daltons; and
heating said mixture to allow said mixture to react to cause a portion of said lignin to degrade.

14. A method in accordance with claim 13 further comprising pressurizing said mixture with an oxygen-containing gas.

15. A method in accordance with claim 14 wherein the oxygen partial pressure is in the range of between about 0.38 to about 1.48 MPa.

## Patentansprüche

1. Kombination von Additiven zur Verwendung in einer Aufhellungsstufe von Pulpen, die weniger als 18 % Lignin enthalten, wobei die Kombination umfasst: eine wässrige Natriumsilicatlösung, ein alkalisches Mittel, das in ausreichender Menge zugesetzt wird, um einen pH der Lösung auf mindestens etwa 8 zu halten, und eine Magnesiumverbindung, die in der Lösung dissoziiert, um Mg(OH)⁺-Kationen zu bilden, wobei die Magnesiumverbindung in einer Menge zugesetzt wird, um zusammen mit etwaigem anderem dissoziierten Magnesium ein Massenverhältnis von Mg zu SiO₂ zwischen etwa 1 : 15 und etwa 1 : 2 zu erreichen, und wobei mindestens 25 % der Silicate ein Molekulargewicht von mindestens 10.000 Dalton haben.

2. Kombination von Additiven gemäß Anspruch 1, wobei das Massenverhältnis von Mg zu SiO₂ zwischen etwa 1 : 15 und etwa 1 : 3 liegt.

3. Kombination von Additiven gemäß Anspruch 1, wobei das alkalische Mittel in ausreichender Menge zugesetzt wird, um den pH der Lösung in einem Bereich von etwa 8 bis etwa 12 zu halten.

4. Kombination von Additiven gemäß Anspruch 1, wobei die Magnesiumverbindung Magnesiumsulfat ist, das als MgSO₄ oder MgSO₄·7H₂O zugesetzt wird.

5. Kombination von Additiven gemäß Anspruch 1, wobei
die wässrige Natriumsilicatlösung in einer Menge zugesetzt wird, dass bezogen auf die Pulpe, eine Konzentration von etwa 0,14 % bis etwa 1,4 % SiO₂ erreicht wird,
und die Magnesiumverbindung in einer Menge zugesetzt wird, dass, bezogen auf die Pulpe, eine Konzentration von etwa 0,01 % bis etwa 0,2 % Mg erreicht wird.

6. Kombination von Additiven gemäß Anspruch 5, wobei
die wässrige Natriumsilicatlösung in einer Menge zugesetzt wird, dass, bezogen auf die Pulpe, eine Konzentration von etwa 0,28 % bis etwa 1,12 % SiO₂ erreicht wird,
und die Magnesiumverbindung in einer Menge zugesetzt wird, dass, bezogen auf die Pulpe, eine Konzentration von etwa 0,02 % bis etwa 0,2 % Mg erreicht wird.

7. Kombination von Additiven gemäß Anspruch 1, wobei das alkalische Mittel aus der Gruppe, bestehend aus mindestens einem von NaOH, Na₂O, MgO, Mg(OH)₂, K₂O, KOH, CaO und Ca(OH)₂, ausgewählt wird.

8. Kombination von Additiven gemäß Anspruch 1, wobei die Magnesiumverbindung aus der Gruppe, bestehend aus mindestens einem von MgO, MgCl₂, Mg(OH)₂ und MgNO₃, ausgewählt wird.

9. Kombination von Additiven gemäß Anspruch 1, die außerdem Wasserstoffperoxid umfasst.

10. Verwendung einer Kombination nach Anspruch 1 bis 9 in einer Aufhellungsstufe von Pulpen, die weniger als 18 % Lignin enthalten.

11. Verwendung nach Anspruch 10, wobei die Pulpe weniger als 5 % Lignin enthält.

12. Verwendung nach Anspruch 11, wobei die Pulpe weniger als 2 % Lignin enthält.

13. Verfahren zur Aufhellung von Pulpe mit folgenden Schritten:
Vermischen von Pulpe, die weniger als 18 % Lignin enthält, mit Wasserstoffperoxid, einer wässrigen Natriumsilicatlösung, einem alkalischen Mittel, das in ausreichender Menge zugesetzt wird, um den pH der Lösung auf mindestens etwa 8 zu halten, und einer Magnesiumverbindung, die in der Lösung dissoziiert, um Mg(OH)⁺-Kationen zu bilden, wobei die Magnesiumverbindung in einer Menge zugesetzt wird, dass zusammen mit etwaigem anderem dissoziierten Magnesium ein Massenverhältnis von Mg zu SiO₂ zwischen etwa 1 : 15 bis 1 : 2. erreicht wird, um ein Gemisch zu bilden, und wobei mindestens 25 % der Silicate ein Molekulargewicht von mindestens 10.000 Dalton haben, und
Erwärmen des Gemischs, damit das Gemisch reagieren und die Zersetzung eines Teils des Lignins bewirken kann.

14. Verfahren nach Anspruch 13, umfassend außerdem das Unter-Druck-Setzen des Gemischs mit einem sauerstoffhaltigen Gas.

15. Verfahren nach Anspruch 14, bei dem der Sauerstoffpartialdruck im Bereich zwischen etwa 0,38 und etwa 1,48 MPa liegt.

## Revendications

1. Combinaison d'additifs pour utilisation dans une étape de blanchiment de pâtes contenant moins de 18 % de lignine, ladite combinaison comprenant : une solution aqueuse de silicate de sodium ; un agent alcalin ajouté en une quantité suffisante pour maintenir le pH de ladite solution à au moins environ 8 ; et un composé du magnésium qui se dissocie dans ladite solution pour former des cations Mg(OH)⁺, ledit composé du magnésium étant ajouté en une quantité permettant d'arriver, avec tout autre magnésium dissocié, à un rapport en masse Mg:SiO₂ compris entre environ 1:15 et environ 1:2, et au moins 25 % des silicates ayant une masse moléculaire d'au moins 10 000 daltons.

2. Combinaison d'additifs selon la revendication 1, dans laquelle ledit rapport en masse Mg:SiO₂ est compris entre environ 1:15 et environ 1:3.

3. Combinaison d'additifs selon la revendication 1, dans laquelle ledit agent alcalin est ajouté en une quantité suffisante pour maintenir le pH de ladite solution dans la plage d'environ 8 à environ 12.

4. Combinaison d'additifs selon la revendication 1, dans laquelle ledit composé du magnésium est le sulfate de magnésium, ajouté sous forme de MgSO₄ ou de MgSO₄.7H₂O.

5. Combinaison d'additifs selon la revendication 1, dans laquelle ladite solution aqueuse de silicate de sodium est ajoutée en une quantité permettant d'arriver à une concentration d'environ 0,14 à environ 1,4 % de SiO₂ par rapport à la pâte ; et ledit composé du magnésium est ajouté en une quantité permettant d'arriver à une concentration d'environ 0,01 à environ 0,2 % de Mg par rapport à la pâte.

6. Combinaison d'additifs selon la revendication 5, dans laquelle ladite solution aqueuse de silicate de sodium est ajoutée en une quantité permettant d'arriver à une concentration d'environ 0,28 % à environ 1,12 % de SiO₂ par rapport à la pâte ; et ledit composé du magnésium est ajouté en une quantité permettant d'arriver à une concentration d'environ 0,02 à environ 0,2 % de Mg par rapport à la pâte.

7. Combinaison d'additifs selon la revendication 1, dans laquelle ledit agent alcalin est choisi dans l'ensemble comprenant au moins l'un des agents NaOH; Na₂O, MgO, Mg(OH)₂, K₂O, KOH, CaO et Ca(OH)₂.

8. Combinaison d'additifs selon la revendication 1, dans laquelle ledit composé du magnésium est choisi dans l'ensemble comprenant au moins l'un des composés MgO, MgCl₂, Mg(OH)₂ et MgNO₃.

9. Combinaison d'additifs selon la revendication 1, qui comprend en outre du peroxyde d'hydrogène.

10. Utilisation d'une combinaison selon l'une quelconque des revendications 1 à 9 dans une étape de blanchiment de pâtes contenant moins de 18 % de lignine.

11. Utilisation selon la revendication 10, pour laquelle ladite pâte contient moins de 5 % de lignine.

12. Utilisation selon la revendication 11, pour laquelle ladite pâte contient moins de 2 % de lignine.

13. Procédé pour blanchir une pâte, qui comprend les étapes consistant :
à mélanger à une pâte contenant moins de 18 % de lignine du peroxyde d'hydrogène, une solution aqueuse de silicate de sodium ; un agent alcalin ajouté en une quantité suffisante pour maintenir le pH de ladite solution à au moins environ 8 ; et un composé du magnésium qui se dissocie dans ladite solution pour former des cations Mg(OH)⁺, ledit composé du magnésium étant ajouté en une quantité permettant d'arriver, avec tout autre magnésium dissocié, à un rapport en masse Mg:SiO₂ compris entre environ 1:15 et environ 1:2, pour former un mélange, et au moins 25 % des silicates ayant une masse moléculaire d'au moins 10 000 daltons ; et
à chauffer ledit mélange pour permettre audit mélange de réagir de façon à amener une partie de ladite lignine à se dégrader.

14. Procédé selon la revendication 13, qui comprend en outre la mise sous pression dudit mélange avec un gaz oxygéné.

15. Procédé selon la revendication 14, dans lequel la pression partielle d'hydrogène est comprise dans la plage d'environ 0,38 à environ 1,48 MPa.
